

1

3,375,122

**INERT AMMUNITION FILLER COMPOSITION  
COMPRISING AN ALUM**

Milton Roth, Rockaway, N.J., assignor to the United States of America as represented by the Secretary of the Army  
No Drawing. Filed Nov. 4, 1966, Ser. No. 592,682  
9 Claims. (Cl. 106—204)

**ABSTRACT OF THE DISCLOSURE**

Dimensionally stable inert practice ammunition fillers which are compatible with high explosives, comprising, in the main, alums combined with cellulose or dextrin to lower the overall specific gravity of the alum combination, and with  $\text{BaSO}_4$  or  $\text{Fe}_2\text{O}_3$  to raise the overall specific gravity of the alum combination.

This invention relates to new compositions of matter and more particularly concerns practice ammunition having improved inert fillers which provide excellent dimensional stability characteristics.

Prior art practice ammunition generally contain a wax or other organic material such as polychlornaphthalene or castorwax which are non-crystalline, soften long before melting and expand and contract extensively with changes in temperature. Poor dimensional stability and strength characterize these waxes or organic compounds. Further, their coefficients of thermal expansion are such that, upon cooling, the filler material shrinks from the shell walls and provide a loose charge having poor and non-reproducible ballistic properties. Additionally, polychlornaphthalene based filler materials are toxic in nature.

In bombs, shells, and the like, used for practice ammunition, high explosive charges are replaced by an inert material which duplicates the weight of the explosive. In addition to having the proper weight for the volume occupied, the inert material should be capable of being loaded in the same manner and, desirably, with the same equipment used for explosives. In order to meet these requirements, the material should melt between 75° and 100° C. Furthermore, to permit reuse of the metal parts, the inert filler must be amenable to ready removal by washing with steam or hot water. The filler material should form a homogeneous mass upon cooling which will be free of voids, and yet readily admit of composition variations such that desired specific gravities from about 1.4 to 2.0 can easily and economically be attained. Most important, the inert material must have dimensional stability to prevent loose charges, exudation, or distortion of the container due to temperature changes. After meeting these requirements, it would be most desirable if the unit cost of the material was relatively low since very large quantities will be used. Finally, the filler material should be non-toxic, odorless, and compatible with such well-known high explosives as RDX (cyclotrimethylenetrinitramine), HMX (cyclotetramethylenetrinitramine) and TNT (2,4,6-trinitrotoluene).

It is, therefore, the principal object of this invention to provide compositions of matter having the aforementioned advantages.

Another object of the invention is to provide inert fillers for practice ammunition having the aforementioned advantages.

Other objects and features of the invention will become apparent as the invention is more fully hereinafter disclosed.

In accordance with these objects, it has been discovered that certain inorganic compounds, such as alums, will combine with cellulose, to yield an inert filler having a

2

lower specific gravity than the alum, or with  $\text{BaSO}_4$  to yield an inert filler having a higher specific gravity than the alum, and yet fulfilling the advantages contemplated by the invention.

The following table illustrates the variations and compositions required to produce a specific gravity range that will be characteristic of a variety of explosives:

TABLE I.—PERCENTAGES OF INERT FILLER FOR VARYING SPECIFIC GRAVITIES

|    | Composition, Wt. Percent                                  |           | Specific Gravity |
|----|-----------------------------------------------------------|-----------|------------------|
|    | $\text{AlNH}_4(\text{SO}_4)_2 \cdot 12\text{H}_2\text{O}$ | Cellulose | $\text{BaSO}_4$  |
| 10 | 100                                                       | -----     | 1.64             |
| 15 | 95                                                        | 5         | 1.58             |
|    | 90                                                        | 10        | 1.50             |
|    | 90                                                        | -----     | 1.71             |
|    | 85                                                        | 15        | 1.77             |
|    | 80                                                        | 20        | 1.85             |
|    | 75                                                        | 25        | 1.95             |

If desired, greater ranges or intermediate values may readily be obtained by one skilled in the art by varying the percentages above.

The ammonium alum is preferably rice to nut size and will have a melting point of about 93.5° C. The cellulose is a powdered, purified, wood type having a moisture content between a 5 to 7%, a maximum of 1% being retained on a 35 mesh screen and a minimum of 96% passing through a 100 mesh screen (U.S. Standard Sieve). The  $\text{BaSO}_4$  should have a specific gravity of about 4.40 and about 99.5% should pass through a 325 mesh screen (U.S. Standard Sieve).

Inorganic ingredients other than ammonium alum may be satisfactorily employed, a number of which are tabulated below:

TABLE II.—COMPOUNDS USEFUL FOR INERT FILLERS

|    | Compound                                                     | Melting Point, °C. | Specific Gravity |
|----|--------------------------------------------------------------|--------------------|------------------|
| 35 | $\text{AlK}(\text{SO}_4)_2 \cdot 12\text{H}_2\text{O}$       | 92                 | 1.76             |
| 40 | $\text{Mg}(\text{NO}_3)_2 \cdot 6\text{H}_2\text{O}$         | 95                 | 1.64             |
|    | $\text{Na}_2\text{B}_4\text{O}_7 \cdot 10\text{H}_2\text{O}$ | 75                 | 1.73             |
|    | $\text{FeSO}_4 \cdot 7\text{H}_2\text{O}$                    | 64                 | 1.61             |
|    | $\text{Al}_2(\text{SO}_4)_3 \cdot 18\text{H}_2\text{O}$      | 86.5               | 1.61             |

$\text{AlK}(\text{SO}_4)_2 \cdot 12\text{H}_2\text{O}$  is somewhat inferior to ammonium alum because the specific gravity is slightly less representative of explosives contemplated by this invention.

In lieu of cellulose, dextrin may be used advantageously to yield an inert filler having a lower specific gravity than the ammonium alum and  $\text{Fe}_2\text{O}_3$  may replace  $\text{BaSO}_4$  to provide an inert filler having a higher specific gravity than the ammonium alum.

50 In those instances where an undesirable chemical reaction may occur between the reactants and the cartridge casing, a corrosion inhibitor such as thiourea, octadecylamine, polyethanol, rosinamine D, and the like, may be incorporated with the reactants in a proportion of about 0.5 to 1.0 parts inhibitor to 100 parts of ammonium alum or its substitute.

55 Since certain applications for inert filler require contact with explosives, compatibility tests were conducted with many of the most widely and frequently used types. I have determined that any explosive based on TNT, RDX, or HMX may satisfactorily and safely be used in contact with my inert filler.

60 In the preparation of my inventive inert fillers, the ammonium alum will be melted by heating to about 100° C. in a stainless steel, glass, copper or other suitable vessel fitted with a mixer. If a stainless steel kettle is used for melting and mixing, a solution containing one part  $\text{CuSO}_4 \cdot 5\text{H}_2\text{O}$  in four to six parts water for each 100 parts of ammonium alum must be used. Apply heat, by any suitable means, to the kettle containing the solution, start the mixer, and allow the inside walls of the kettle to be wetted with the solution. If glass, plastic, copper, or lead-

lined equipment is used, addition of the copper sulfate solution may be omitted. Aluminum kettles should not be used unless they are coated with a paint free from iron oxide, zinc oxide or aluminum. Throughout the melting and mixing, the kettle should be opened only while material is being added in order to minimize evaporation of the steam that is evolved.

Now add the desired weight of alum, or its substitute, rather slowly to the heated kettle containing the copper sulfate solution so that the mixer will not become overloaded. When all the alum has been added, continue the heating and stirring in the closed vessel until a clear liquid is obtained. Open the kettle, add the cellulose or barium sulfate as rapidly as possible, again close the opening and continue mixing until a uniform dispersion appears to be obtained. Generally, this will require not more than five minutes. Add the required weight of corrosion inhibitor, if necessary, replace the cover and mix for two to three minutes. The temperature of the mixture should be about 95° C.

Pour the mixture into shells or bombs which have previously been coated on their inner surfaces with an acid proof black paint or some other suitable coating which will prevent reaction of the molten mixture with the cartridge casing. Finally, allow the mixture to cool slowly to room temperature.

It is apparent from the foregoing description that I have provided new compositions of matter ideally suited for inert fillers for use in practice ammunition, the inert filler being dimensionally stable over a wide range of temperature, low in cost, non-toxic, odorless, water soluble and compatible with HMX, RDX and TNT. The specific gravity of the filler can be readily adjusted to simulate any explosive composition. Existing melting and cast loading equipment may still be used. Rapid solidification with low shrinkage expedites the filling of bombs and shells. The low viscosity of the molten filler assures complete conformity to the shape of the container into which it is poured and the dimensional stability characteristics of my composition assures adhesion to the walls of the article or container within a temperature range of about -70° to 190° F. Clean-up and disposal of excess filler is simple and rapid since it can readily be dissolved and be washed away with hot water or steam.

My compositions are expected to lend themselves to other applications, such, for example, as in ballasts, molds and models wherein a hard, castable, dimensionally stable, inexpensive material of varying densities and colors might be desired.

I claim:

1. A practice ammunition filler of a substantially inert composition of matter dimensionally stable over a temperature range of about -70° to 190° F. and capable of yielding specific gravities within limits of about 1.50 to 1.95, said composition comprising:

an aluminum alum and a material for changing specific gravity of said aluminum alum to a value within said limits selected from the group consisting of cellulose, dextrin, BaSO<sub>4</sub> and Fe<sub>2</sub>O<sub>3</sub> to produce said inert composition.

2. An inert composition as described in claim 1, said

composition having a specific gravity of about 1.58 and comprising about 95 weight percent AlNH<sub>4</sub>(SO<sub>4</sub>)<sub>2</sub>·12H<sub>2</sub>O and about 5 weight percent of cellulose.

3. An inert composition as described in claim 1, said composition having a specific gravity of about 1.50 and comprising about 90 weight percent of



and about 10 percent cellulose.

4. An inert composition as described in claim 1, said composition having a specific gravity of 1.71 and comprising about 90 weight percent of AlNH<sub>4</sub>(SO<sub>4</sub>)<sub>2</sub>·12H<sub>2</sub>O and about 10 weight percent barium sulfate.

5. An inert composition as described in claim 1, said composition having a specific gravity of about 1.77 and comprising about 85 weight percent of



and about 15 weight percent barium sulfate.

6. An inert composition as described in claim 1, said composition having a specific gravity of about 1.85 and comprising about 80 weight percent of



and about 20 weight percent barium sulfate.

7. An inert composition as described in claim 1, said composition having a specific gravity of about 1.95 and comprising about 75 percent by weight of



and about 25 weight percent barium sulfate.

8. A practice ammunition filler of a substantially inert composition of matter dimensionally stable over a temperature range of about -70° to 190° F. and capable of yielding specific gravities within limits of about 1.50 to

1.95, said composition comprising:  
an inorganic compound selected from the group consisting of AlNH<sub>4</sub>(SO<sub>4</sub>)<sub>2</sub>·12H<sub>2</sub>O, AlK(SO<sub>4</sub>)<sub>2</sub>·12H<sub>2</sub>O, Mg(NO<sub>3</sub>)<sub>2</sub>·6H<sub>2</sub>O, Na<sub>2</sub>B<sub>4</sub>O<sub>7</sub>·10H<sub>2</sub>O, FeSO<sub>4</sub>·7H<sub>2</sub>O and Al<sub>2</sub>(SO<sub>4</sub>)<sub>3</sub>·18H<sub>2</sub>O combined with a material for changing specific gravity of said inorganic compound to a value within said limits selected from the group consisting of cellulose, dextrin, BaSO<sub>4</sub> and Fe<sub>2</sub>O<sub>3</sub> to produce said inert composition, and about 0.5 to 1.0 part corrosion inhibitor per 100 parts of said inorganic compounds, said corrosion inhibitor being an organic nitrogen compound.

9. The composition of claim 8 wherein said corrosion inhibitor is selected from the group consisting of thiourea, octadecylamine, and polyethanol rosinamine D.

#### References Cited

#### UNITED STATES PATENTS

3,018,203 1/1962 Guth ----- 149—45 X  
55 3,108,917 10/1963 McIrvine ----- 149—105 X

CARL D. QUARFORTH, Primary Examiner.

BENJAMIN R. PADGETT, Examiner.

S. J. LECHERT, JR., Assistant Examiner.